

1

3,484,184

## HALOALKYL PHOSPHINIC ACIDS AND THEIR APPLICATION TO COTTON

Leon H. Chance and Ethel K. Leonard, New Orleans, and  
George L. Drake, Jr., Metairie, La., assignors to the  
United States of America as represented by the Secretary  
of Agriculture

No Drawing. Filed May 3, 1967, Ser. No. 635,680  
Int. Cl. D06m 13/30, 13/44

U.S. Cl. 8—120

11 Claims

### ABSTRACT OF THE DISCLOSURE

Bis(chloromethyl)phosphinic acid is prepared by a new method; other phosphinic acids are prepared by reacting certain ketones with hypophosphorus acid; and new cellulosic derivatives are prepared by crosslinking fibrous cellulose with these phosphorus containing compounds.

A non-exclusive, irrevocable, royalty-free license in the invention herein described throughout the world for all purposes of the United States Government, with the power to grant sublicenses for such purposes, is hereby granted to the Government of the United States of America.

This invention relates to haloalkyl phosphinic acids, to the preparation thereof, and to a process for imparting improved physical and chemical properties to cellulosic textiles by treating said cellulosic textiles with the organophosphorus compounds of this invention. More specifically this invention relates to the preparation of a known phosphinic acid by a new method, to the preparation of two new compounds by another method, and to the utilization of these compounds in textile applications which would yield goods with wet wrinkle resistance, cation-exchange properties, fire-retardance, and other useful properties.

The main object of the instant invention is to provide a process for imparting to cotton and other cellulosic textiles improved wet wrinkle recovery.

A second object of the instant invention is to provide a process for imparting to cotton and other cellulosic textiles cation-exchange properties.

A third object of the instant invention is to provide a process for improving the comfort factor of garments made from cotton and other cellulosic textiles by providing the treated textile with increased moisture regain.

A fourth object of the instant invention is to provide textiles with reduced combustibility as an additional physical factor obtained in the finished goods together with the imparted comfort factor.

A fifth object of the instant invention is to provide new methods of preparing phosphorus-containing compounds which also contain active halogen groups.

A sixth object of the instant invention is to provide a new method of preparing known and useful compounds.

A seventh object of the instant invention is to disclose the new phosphinic acid type compounds produced by processes of the instant invention.

Searching the prior art we find that acetone reacts with hypophosphorus acid to produce bis(1-hydroxyisopropyl)phosphinic acid (Beilstein I, 652 (1918)). The reaction requires several days of refluxing, and rather low yields are obtained. K. M. Moedritzer (J. Amer. Chem. Soc. 83, 4381—4 (1961)) prepared bis(chloromethyl)phosphinic chloride by a complex four step reaction. G. L. Drake, Jr., et al. (U.S. Patent 2,979,374) reacted chloromethyl phosphinic acid with fibrous cellulose in the presence of alkali to produce phosphonomethylated cellulosic materials having reduced combustibility and cation-exchange properties. Cotton fabrics treated with chloromethyl phosphinic

2

acid, however, do not have improved wrinkle resistance and do have a slick feel when wet with water.

In accordance with one aspect of the present invention, it has been found that when halogen substituted acetones—such as chloroacetone and dichloroacetone—are used the reaction proceeds rapidly and with good yields. This may be attributed to the activating influence of the halogens on the carbonyl groups of the acetone. In reference to the complex, four step reaction of Moedritzer, the present process differs in that we prepare the bis(chloromethyl)phosphinic acid by a simple new process with good yields wherein bis(hydroxymethyl)phosphinic acid is reacted with thionyl chloride, and the resulting phosphinic chloride is then hydrolyzed with water.

In the course of investigation we have also found that phosphinic acids having the graphic formula



where X represents either hydrogen or a halogen, and Y represents a halogen, can be prepared by reacting hypophosphorus acid with haloacetones having the graphic formula



where X and Y are members of the group halogen and hydrogen, with the proviso that when one is hydrogen the other must be halogen.

We have also found that phosphinic acids of the graphic formula



where X represents a halogen, can be prepared by reacting bis(hydroxymethyl)phosphinic acid with a suitable halogenating agent such as  $\text{SOX}_2$ ,  $\text{PX}_3$ , or  $\text{PX}_5$ , where X represents a halogen atom, followed by hydrolysis of the resulting phosphinic halide.

We have further found that the sodium salt of the compound bis(iodomethyl)phosphinic acid can also be prepared by reacting bis(chloromethyl)phosphinic acid with sodium iodide in a suitable solvent.

In accordance with the present invention the reaction of hypophosphorous acid with the haloacetones is carried out by heating crystalline hypophosphorous acid with an excess of the haloacetone without the use of a solvent. Although organic solvents, such as methanol, ethanol, or isobutanol, may be used in the reaction the preferred procedure is to carry out the reaction without a solvent because higher yields are obtained in this manner; and bis(chloromethyl)phosphinic acid is prepared by reacting crystalline bis(hydroxymethyl)phosphinic acid with an excess of thionyl chloride without the use of a solvent.

The reaction with cellulosic material takes place between the cellulosic hydroxyl groups and the halogen atoms of the alkali metal salts of the haloalkyl phosphinic acids, thereby crosslinking the cellulose through stable ether linkages. Cellulose crosslinks are shown by insolubility of the cellulose in aqueous 0.5 molar cupriethylene-diamine hydroxide. The resulting alkali metal cellulose phosphinate can be converted to the corresponding phosphinic acid by soaking the cellulose phosphinate in a dilute solution of a strong mineral acid until all of the alkali metal atoms have been replaced by hydrogen atoms. These hydrogen atoms can be replaced by other cations by immersing in the appropriate solution containing the desired cation. When the cation is ammonium ion the cellulosic material has a greater reduction in combustibility than any other cation.

Cotton fibers, regenerated cotton fibers, paper, or other cellulosic materials are suitable for this invention. Cotton fiber is the preferred material, and may be in the form of fibers, sliver, yarn, or fabric, but yarn or fabric is preferred..

The reaction with cellulosic material can be carried out by using the metal salt of chloroalkyl phosphinic acids. However, the invention is not limited to the chloro derivatives. Other halogen derivatives can be used.

The aqueous solutions suitable for use in the invention can be aqueous solutions of the haloalkylphosphinic acid and any metal hydroxide or alkali metal carbonate containing about from 2% to 20% by weight of unreacted alkali metal hydroxide or carbonate and about from 5% to 25% by weight of the haloalkylphosphinic acids. Preferred concentrations of alkali metal hydroxide or carbonate and phosphinic acid depends on the phosphinic acid being used and on the degree of cellulosic crosslinking desired. It is preferable to use the solutions while they are fresh, because the longer the solutions stand, the less efficient the reaction becomes.

The reaction of the chloroalkyl phosphinic acids with cellulosic materials may be carried out by impregnating the cellulosic material with an aqueous alkali metal hydroxide or carbonate, in excess of that required to neutralize the acid, drying, and then impregnating the dried cellulosic material with an aqueous solution of the phosphinic acid, and finally curing the cellulosic material at temperatures ranging about from 110° C. to 175° C., for periods of time ranging about from 5 minutes to 30 minutes. The preferred method of carrying out the reaction involves impregnating the textile in only one aqueous solution. The chloroalkyl phosphinic acid is dissolved in aqueous alkali metal hydroxide or carbonate in excess of that required to neutralize the acid. Sodium hydroxide and sodium carbonate are preferred. The cellulosic material is impregnated with the solution, dried, and cured at temperatures ranging about from 110° C. to 175° C. for periods of time about from 5 minutes to 30 minutes, the longer times being used with the lower temperatures. When alkali metal hydroxides are used the preferred curing temperatures are in the range of about from 140° to 150° C. for about from 5 to 10 minutes. When the alkali metal carbonates are used the preferred curing temperatures are in the range of about from 165° to 175° C. for periods of time of about from 5 to 10 minutes.

The fibrous cellulosic material can be impregnated and heated by any apparatus conventionally used for processing such materials.

The following examples illustrate procedures that have been used successfully in carrying out the invention and are not meant as a limitation thereof. Cotton fabrics which have been treated by process of this invention were tested by the standard methods recommended by the American Society for Testing Materials, Philadelphia, Pa., Committee D-13. Wet and dry wrinkle recovery were determined by the Monsanto Method, ASTM D1424-59; and moisture regain by ASTM D629-5019. Fabric combustibility tests were carried out in this manner: The fabric samples were cut into strips 1 cm. x 5 cm., and each strip being tested was held with the surface vertical to the flame, and the long edge at the indicated angle from vertical, and ignited at the specific points. Observations were made to see whether or not the burning would continue along the strip and to determine the presence or absence of an afterglow. Equivalent weights were determined by standard titration procedures. All percentages and parts in the examples are by weight.

#### PREPARATION OF PHOSPHINIC ACIDS

Example 1.—Bis(1-hydroxy 2-chloroisopropyl)phosphinic acid

*Method I.*—Crystalline hypophosphorous acid (33.0 grams, 0.5 mole) was dissolved in chloro-2-propanone (185.0 grams, 2.0 moles). The solution was heated on a

water bath for 15½ hours at about 80° C. During the heating period the reaction mixture turned black and crystallized to a solid mass. The mass was slurried vigorously with 300 ml. of benzene to remove the black material, and the crystals were filtered. Additional crystals were recovered from the benzene filtrate by evaporation of the greater part of the benzene. The crystals were slurried again with 150 ml. of benzene containing 5 ml. of ethanol. The total crude yield was 72.3 grams or 57.6% based on the hypophosphorus acid. M.P. of the crude product was 149-159° C. (corrected).

Purer crystals with an M.P. of 150-151° C. were obtained by stirring the crude crystals with a mixture of hot benzene and ethanol in a ratio of 30:1, cooling, filtering, and washing the white crystals on filter with acetonitrile. Analytically pure crystals were obtained by recrystallization from a mixture of benzene and ethanol. The crystals had a M.P. of 153.5-154.5° C. (corr.).

Elemental analysis.—Calcd. for  $C_6H_{13}O_4Cl_2P$ : C, 28.72; H, 5.19; Cl, 28.25; P, 12.34; equivalent weight, 250.93. Found: C, 29.03; H, 5.37; Cl, 27.47; P, 11.57; equivalent weight, 247.91.

The compound is soluble in water, alcohol, and acetone.

*Method II.*—Crystalline hypophosphorus acid (16.5 grams, 0.25 mole) and chloro-2-propanone (50.0 grams, 0.54 mole) were dissolved in 100 ml. of isobutanol. The solution was heated at 95-100° C. for 16 hours. The isobutanol was removed by vacuum distillation, leaving a viscous brown residue which partially crystallized. To this brown mass was added 150 ml. of benzene. The dark viscous material dissolved, leaving the crystals undissolved. The crystals were filtered and washed with benzene. They were white and weighed 6.5 grams. When recrystallized from a mixture of benzene and ethanol, the compound had a melting point of 153.5-154.5° C. and was identical with that obtained by Method I.

Example 2.—Bis(1-hydroxy 2,2'-dichloroisopropyl)-phosphinic acid

1,3-dichloro-2-propanone (63.5 grams, 0.5 mole) and crystalline hypophosphorus acid (13.2 grams, 0.2 mole) were mixed and heated to 50° C. The crystals melted and were stirred to make a homogeneous solution. Heating at 50° C. was continued for 15½ hours. During this time the reaction mixture solidified to a white crystalline mass. The mass was broken up and stirred successively with two 50 ml. portions of hot benzene to remove unreacted materials. The white crystals weighed 56.7 grams. Additional crystals (1.6 grams) were recovered from the benzene to make a total yield of 58.3 grams or 91%. The crystals had a M.P. of 137-139° C. (corrected) and was pure enough for use in examples cited below. Recrystallization from a benzene and ethanol mixture produced an analytical sample with a melting point of 141-142° C. (corrected).

Elemental analysis.—Calcd. for  $C_6H_{11}O_4Cl_4P$ : C, 22.52; H, 3.47; Cl, 44.32; P, 9.68. Found: C, 22.91; H, 3.64; Cl, 43.54; P, 8.90.

Determination of the equivalent weight could not be determined by direct titration with 0.1 N NaOH, because the chlorine atoms were active enough to hydrolyze during the titration. Therefore, the compound was heated in an excess of standard 0.1 N NaOH for 2½ hours at 65-70° C. to hydrolyze all four chlorine atoms. The solution was then back titrated with standard 0.1 N HCl. The calculated equivalent weight by this method is one-fifth of the molecular weight, or 63.97. The equivalent weight found by the above method was 62.15.

The compound is soluble in water, alcohol, and acetone.

Example 3.—Bis(chloromethyl)phosphinic acid

*Step 1.*—Thionyl chloride (416.5 grams, 3.5 mole) was placed in a 3-neck flask equipped with a stirrer and a reflux condenser topped with a drying tube to exclude

moisture. Bis(hydroxymethyl) phosphinic acid (126.0 grams, 1.0 mole) was melted and added gradually to the stirred flask. The reaction was endothermic, the flask becoming cold during the additions. After the addition was complete, the reaction mixture was allowed to stand overnight. The excess thionyl chloride was removed by distillation. The crude bis(chloromethyl) phosphinic chloride was a liquid and weighed 170 grams, a 93.7 yield based on bis(hydroxymethyl) phosphinic acid.

Step 2.—Crude bis(chloromethyl) phosphinic chloride (170.0 grams, 0.94 mole) was dissolved in 265 ml. of benzene, and added dropwise over a 30 minute period to a vigorously stirred flask containing 395 ml. of benzene and 20 grams (1.0 mole) of water. Stirring was continued for 6 hours at room temperature, and finally the mixture was refluxed for one hour. The flask was cooled in an ice water bath, and the crystals which separated were filtered and dried. The crude yield of bis(chloromethyl) phosphinic acid was 100%, but melted over a range of 75–79° C. The crude crystals were stirred with a mixture of 240 ml. of benzene and 60 ml. of acetone, cooled in ice water, and filtered. The recovery was 73% of white crystals with a M.P. of 77–80° C. Crystals melting at 80.5–81.5° C. were obtained by repeating the purification step. Additional crystals were obtained from the combined benzene-acetone filtrates to give a total yield of pure crystals of 69%. The melting point (80.5–81.5° C.,

## APPLICATION TO COTTON FABRIC

In all of the following examples 80 x 80 mercerized cotton printcloth was used. The fabric was immersed in the solution and the excess squeezed out by passing through squeeze rolls to a wet pickup of 85–100% depending on solution concentrations. The fabric was then dried and cured without tension unless otherwise stated, and finally washed and dried.

For brevity, the phosphinic acids will be designated as follows: bis(1-hydroxy - 2 - chloroisopropyl) phosphinic acid—HCPA; bis(1-hydroxy 2,2'-dichloroisopropyl) phosphinic acid—HDPA; and bis(chloromethyl) phosphinic acid—BCPA.

## Example 5.—HCPA-NaOH catalyst

Solutions were prepared by dissolving HCPA in aqueous NaOH solutions of the concentrations indicated in Table I, while keeping the solution cool to prevent spontaneous heating up. All solutions contained 15% HCPA. Cotton fabric samples were treated with freshly prepared solutions, as well as with solutions aged from 2 to 24 hours to demonstrate solution stability. Fabric samples, after impregnation, were dried for 5 minutes at 85° C. and cured for 5 minutes at 140° C., washed and dried. Fabric data are shown in Table I. Very slight fabric discoloration was completely removed by a mild chlorine bleach.

TABLE I

| NaOH conc., percent | Age of soln., hrs. | Phosphorus content, percent | Wrinkle recovery (degrees) |     | Moisture regain, percent | Cation-exchange capacity, meq./gm. |
|---------------------|--------------------|-----------------------------|----------------------------|-----|--------------------------|------------------------------------|
|                     |                    |                             | Wet                        | Dry |                          |                                    |
| 7.5                 | Fresh              | 0.06                        | 232                        | —   | —                        | —                                  |
| 11.0                | Fresh              | 0.77                        | 264                        | —   | —                        | —                                  |
| 15.0                | Fresh              | 0.98                        | 235                        | 201 | 10.41                    | 0.295                              |
| 15.0                | 2                  | 0.85                        | 236                        | 196 | 10.32                    | 0.286                              |
| 15.0                | 4                  | 0.72                        | 234                        | 189 | 10.30                    | 0.222                              |
| 15.0                | 24                 | 0.35                        | 221                        | 178 | 9.84                     | 0.087                              |
| 20.0                | Fresh              | 0.95                        | 221                        | 193 | 11.30                    | —                                  |
| 20.0                | 2                  | 0.75                        | 230                        | 180 | 10.94                    | —                                  |
| 25.0                | Fresh              | 0.89                        | 224                        | 192 | 11.76                    | —                                  |
| 25.0                | 2                  | 0.63                        | 228                        | 185 | 11.14                    | —                                  |
| Untreated fabric    |                    |                             | 198                        | 191 | 7.48                     | 0.05                               |

corrected) agreed with that of bis(chloromethyl) phosphinic acid prepared by a different method in the literature.

Elemental analysis.—Calcd. for  $C_2H_5O_2Cl_2P$ : C, 14.74; H, 3.09; Cl, 43.52; P, 19.01; equivalent weight, 162.89. Found: C, 14.81; H, 3.11; Cl, 43.56; P, 19.10; equivalent weight, 160.30.

The compound was soluble in water, alcohol, and acetone.

## Example 4.—Bis(iodomethyl) phosphinic acid, sodium salt

Bis(chloromethyl) phosphinic acid (16.3 g.) was dissolved in acetone (75 ml.) and added to a flask containing sodium iodide (39.0 grams) in acetone (175 ml.). The mixture was refluxed with stirring for about 12 hours. The precipitated sodium chloride was filtered. The filtrate was cooled to about -10° C. The crystals which separated were filtered and washed with cold acetone. Pale yellow crystals (5.5 grams) were obtained. The acetone filtrate was evaporated to about 30 ml. volume. Black crystals were obtained. The black color was due to the presence of free iodine. The crystals were washed with absolute ethanol (50 ml.). Pale yellow crystals (1.8 grams) were obtained. Total crude yield was 7.3 grams. Lustrous white crystals were obtained by recrystallization from water-ethanol (1:4 volume ratio). The product was largely the sodium salt of bis(iodomethyl) phosphinic acid.

Elemental analysis.—Calcd. C, 6.53%; H, 1.10%; I, 69.00%; P, 8.42%. Found: C, 7.66%; H, 1.26%; I, 60.56%; P, 9.65%.

45

Elemental analysis.—Calcd. for  $C_2H_5O_2Cl_2P$ : C, 14.74; H, 3.09; Cl, 43.52; P, 19.01; equivalent weight, 162.89. Found: C, 14.81; H, 3.11; Cl, 43.56; P, 19.10; equivalent weight, 160.30.

A second sample of fabric was treated similarly except it was cured for 30 minutes at 110° C. It had a wet wrinkle recovery angle of 247°, a dry wrinkle recovery angle of 173°, and phosphorus content of 0.77%.

## Example 7

A two-step method was used to apply HCPA to cotton fabric. Two fabric samples were first impregnated with a 25% aqueous solution of NaOH, dried for 5 minutes at 85° C., and then impregnated with a 20% aqueous solution of HCPA. The first sample was cured for 5 minutes at 140° C., washed and dried. The fabric contained 0.82% P. The second sample was cured for 30 minutes at 110° C., washed and dried. It contained 0.73% P.

Example 8.—HCPA-Na<sub>2</sub>CO<sub>3</sub> catalyst

A solution was prepared by dissolving 5.0 g. of HCPA in 45 g. of 15% Na<sub>2</sub>CO<sub>3</sub>. The solution contained 10% HCPA. Three samples of cotton fabric were impregnated with the solution and each dried for 5 minutes at 85° C. The samples were then cured for 5 minutes at tempera-

tures shown in Table II. Wrinkle recovery angles, phosphorus content, and moisture regain are given.

TABLE II

| Curing temp., °C. | Wrinkle recovery (degrees) |     | Moisture regain, percent | Phosphorus content, percent |
|-------------------|----------------------------|-----|--------------------------|-----------------------------|
|                   | Wet                        | Dry |                          |                             |
| 140               | 224                        | 183 |                          | <0.1                        |
| 165               | 237                        | 179 |                          | 0.15                        |
| 175               | 224                        | 187 | 9.25                     | 0.18                        |

The samples cured at 140° C. and 165° C. were soluble in cupriethylenediamine dihydroxide, indicating little or no cross-linking. The sample cured at 175° C. was partially insoluble, indicating a little crosslinking of the cellulose.

## Example 9

Solutions were prepared in the same way as in Example 5 except HDPA was used instead of HCPA. All solutions contained 15% HDPA. Fabric discoloration was greater than when HCPA was used, and therefore required stronger bleaching conditions to remove the color. Fabric data are shown in Table III.

TABLE III

| NaOH conc., percent | Age of soln., hrs. | Phosphorus content, percent | Wrinkle recovery (degrees) |     | Moisture regain, percent | Cation-exchange capacity, meq./g. |
|---------------------|--------------------|-----------------------------|----------------------------|-----|--------------------------|-----------------------------------|
|                     |                    |                             | Wet                        | Dry |                          |                                   |
| 7.0                 | Fresh              | 0.18                        | 243                        |     |                          |                                   |
| 10.5                | Fresh              | 0.86                        | 283                        |     |                          |                                   |
| 12.5                | Fresh              |                             | 283                        | 224 | 8.70                     |                                   |
| 15.0                | Fresh              | 1.13                        | 281                        | 232 | 9.64                     | 0.412                             |
| 15.0                | 4                  | 0.82                        | 267                        | 209 |                          |                                   |
| 15.0                | 24                 | 0.16                        | 229                        | 174 |                          |                                   |
| 20.0                | Fresh              | 1.18                        | 273                        | 216 | 10.39                    | 0.397                             |
| 20.0                | 4                  | 0.49                        | 244                        | 188 |                          |                                   |
| 25.0                | Fresh              | 0.95                        | 293                        | 194 | 11.98                    | 0.373                             |
| 25.0                | 4                  | 0.12                        | 226                        | 174 |                          |                                   |

## Example 10

A two-step method was used to apply HDPA to cotton fabric in the same manner described for the first

angles, phosphorous content, and moisture regain are given in Table IV.

TABLE IV

| Curing temp., °C. | Wrinkle recovery (degrees) |     | Moisture regain, percent | Phosphorus content, percent |
|-------------------|----------------------------|-----|--------------------------|-----------------------------|
|                   | Wet                        | Dry |                          |                             |
| 140               | 252                        | 195 |                          | 0.25                        |
| 165               | 260                        | 208 |                          | 0.44                        |
| 175               | 258                        | 211 | 9.35                     | 0.49                        |

All of the fabric samples were insoluble in aqueous 0.5 molar cupriethylenediamine hydroxide, indicating cross-linking of the cellulose.

## Example 13

Solutions were prepared by dissolving BCPA in aqueous NaOH solution of the concentrations indicated in Table V, keeping the solution cool to prevent heating up due to neutralization of the acid. All solutions contained 10% BCPA. Cotton fabric samples were treated with fresh solutions as well as with solutions aged for 4 hours and 24 hours. Fabric samples, after impregnation were dried

## Example 10

for 5 minutes at 85° C. and cured for 5 minutes at 140° (except for one sample cured for 5 minutes at 165° C.), washed, and dried. Fabric data are shown in Table V.

TABLE V

| NaOH conc., percent | Age of soln., hrs. | Phosphorus content, percent | Wrinkle recovery (degrees) |     | Moisture regain, percent | Cation-exchange capacity, meq./gm. |
|---------------------|--------------------|-----------------------------|----------------------------|-----|--------------------------|------------------------------------|
|                     |                    |                             | Wet                        | Dry |                          |                                    |
| 5.0 <sup>1</sup>    | Fresh              | 0.60                        | 245                        | 195 | 9.00                     |                                    |
| 5.0                 | Fresh              | 0.26                        | 227                        | 184 | 8.69                     | 0.088                              |
| 7.5                 | Fresh              | 0.60                        | 239                        | 193 | 9.25                     | 0.199                              |
| 10.0                | Fresh              | 0.78                        | 256                        | 201 | 10.04                    | 0.254                              |
| 12.5                | Fresh              | 0.72                        | 265                        | 206 | 9.78                     |                                    |
| 15.0                | Fresh              | 0.63                        | 266                        | 200 | 9.40                     | 0.283                              |
| 15.0                | 4                  | 0.78                        | 279                        | 178 |                          |                                    |
| 15.0                | 24                 | 0.50                        | 262                        | 183 |                          |                                    |
| 16.0                | Fresh              | 0.58                        | 286                        |     |                          |                                    |

<sup>1</sup> Cured 5 minutes at 165° C.

sample in Example 7. The fabric contained 0.66% P.

## Example 11

A solution was prepared by dissolving HDPA (3.25 g.) in 15% aqueous NaOH (21.75 g.). Cotton printcloth impregnated with the solution was cured for 30 minutes at 110° C. It had a wet wrinkle recovery angle of 278° C., a dry wrinkle recovery angle of 189°, and a phosphorus content of 0.79%.

Example 12.—HDPA-Na<sub>2</sub>CO<sub>3</sub> catalyst

A solution was prepared in the same manner as in Example 8 except HDPA was used instead of HCPA. Fabric samples were treated as in Example 8. Wrinkle recovery

Very slight fabric discoloration was removed by a mild chlorine bleach.

65

## Example 14

A solution was prepared by dissolving BCPA (2.5 grams) in 15% aqueous NaOH (22.5 grams). Cotton printcloth impregnated with the solution was cured for 30 minutes at 110° C. It had a wet wrinkle recovery angle of 266°, a dry wrinkle recovery angle of 180°, and a phosphorus content of 0.55%.

Example 15.—BCPA-Na<sub>2</sub>CO<sub>3</sub> catalyst

A solution was prepared in the same manner as in Example 8 except BCPA was used instead of HCPA.

75

Fabric samples treated in the same manner as in Example 8. Wrinkle recovery angles, phosphorus content and moisture regain of the fabric samples are given in Table VI.

TABLE VI

| Curing temp., °C. | Wrinkle recovery (degrees) |     | Moisture regain, percent | Phosphorus content, percent |
|-------------------|----------------------------|-----|--------------------------|-----------------------------|
|                   | Wet                        | Dry |                          |                             |
| 140               | 219                        | 173 | -----                    | <0.1                        |
| 165               | 228                        | 182 | -----                    | 0.15                        |
| 175               | 236                        | 184 | 9.53                     | 0.25                        |

The samples which were cured at 165° C. and 175° C. although swelled by aqueous 0.5 molar cupriethylenediamine hydroxide, were insoluble, indicating crosslinking of the cellulose.

## Example 16

Three solutions were prepared as follows: (1) HCPA (6.75 g.) was dissolved in 15% aqueous NaOH (38.25 g.); (2) HDPA (7.5 g.) was dissolved in 15% aqueous NaOH (42.5 g.); (3) BCPA (5.0 g.) was dissolved in 12.5% aqueous NaOH (45.0 g.). Cotton fabric samples were impregnated with each solution, and each sample placed on a pin frame at its original dimensions before impregnation. The fabrics were then dried 5 minutes at 85° C. and cured 5 minutes at 140° C. The pin frame maintained the fabric at constant dimensions during the drying and curing operations. The fabric was removed from the pin frame, washed, replaced on the pin frame, and dried at constant dimensions. Data for the fabric samples are shown in Table VII.

All of the samples were insoluble in aqueous 0.5 molar cupriethylenediamine hydroxide solution. This is an indication that the cellulose is crosslinked.

hydroxide, indicating crosslinking of the cellulose. The fabric contained 0.37% P, and had a wet wrinkle recovery angle of 253°.

We claim:

1. A two-bath process for imparting to cellulosic textiles wet wrinkle recovery, cation-exchange properties, improved moisture regain quality, and reduced combustibility, comprising:

(a) impregnating the cellulosic textile with an aqueous solution containing about 2.0% to 20% alkali metal base selected from the group consisting of sodium hydroxide and sodium carbonate,

(b) drying the wet impregnated textile from (a) for about 5 minutes at about 85° C.,

(c) impregnating the dried textile from (b) with an aqueous 5% to 25% solution containing a phosphinic compound to an 85-100% wet pickup, said phosphinic compound selected from the group consisting of:

bis(1-hydroxy-2,2'-dichloroisopropyl) phosphinic acid,

bis(1-hydroxy-2-chloroisopropyl) phosphinic acid,

bis(iodomethyl) sodium phosphinate, and

bis(chloromethyl) phosphinic acid, and

(d) curing the phosphinic impregnated textile for about from 5 to 30 minutes at temperatures of about from 110° to 175° C., using the longer periods of time with the lower temperatures, then washing and drying the cured textile to obtain a finished product with a phosphorus content of about from 0.06% to 1.58%.

2. The process of claim 1 wherein the alkali metal base is sodium hydroxide and the phosphinic compound is bis(1-hydroxy-2,2'-dichloroisopropyl) phosphinic acid.

TABLE VII

| Compound | Phosphorus content, percent | Cation-exchange, meq./gm. | Wrinkle recovery (W+F) |     | Breaking strength (filling) (lbs.) | Elongation at break (filling) percent | Tearing strength (filling) gms. | Moisture regain percent | Flex abrasion (filling) cycles |
|----------|-----------------------------|---------------------------|------------------------|-----|------------------------------------|---------------------------------------|---------------------------------|-------------------------|--------------------------------|
|          |                             |                           | Wet                    | Dry |                                    |                                       |                                 |                         |                                |
| HCPA     | 0.95                        | 0.321                     | 236                    | 195 | 33.6                               | 19.1                                  | 500                             | 10.6                    | 535                            |
| HDPA     | 1.10                        | 0.414                     | 276                    | 201 | 22.6                               | 23.0                                  | 400                             | 10.3                    | 230                            |
| BCPA     | 0.91                        | 0.278                     | 272                    | 206 | 25.2                               | 26.1                                  | 460                             | 10.1                    | 312                            |
| Control  | -----                       | 0.052                     | 198                    | 191 | 39.1                               | 25.9                                  | 787                             | 7.5                     | 759                            |

## Example 17

Samples of cotton printcloth treated with HCPA, HDPA, and BCPA were tested for flame resistance in the sodium salt form, the acid form, and the ammonium salt form. The sodium form was converted to the acid form by soaking the fabric for about 30 minutes in dilute hydrochloric acid, followed by thorough rinsing in distilled water, and drying. The acid form was converted to the ammonium form by soaking for about 30 minutes in dilute ammonium hydroxide, followed by rinsing in distilled water, and drying. Fabric combustibility test results are shown in Table VIII.

TABLE VIII

| Fabric treatment | Phosphorus content, percent | Strip burn angle, degrees |                      |           |
|------------------|-----------------------------|---------------------------|----------------------|-----------|
|                  |                             | Na salt                   | NH <sub>4</sub> salt | Acid form |
| HCPA             | 1.58                        | 45                        | 90                   | 90        |
| HDPA             | 1.10                        | 0                         | 110                  | 90        |
| BCPA             | 0.72                        | 0                         | 90                   | 90        |

All of the treated samples left a black charred residue with no afterglow. The control fabric burned completely.

## Example 18

Bis(iodomethyl) phosphinic acid (1.0 gram) was dissolved in 5% NaOH (9.0 grams). A sample of cotton printcloth was impregnated with the solution, and the fabric was dried at 85° C. and cured for 5 minutes at 140° C., washed, and dried. Fibers from the fabric were insoluble in aqueous 0.5 molar cupriethylenediamine

70

5

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

## 11

bis(1 - hydroxy-2,2'-dichloroisopropyl) phosphinic acid,  
 bis(1 - hydroxy-2-chloroisopropyl) phosphinic acid,  
 bis(iodomethyl) sodium phosphinate, and  
 bis(chloromethyl) phosphinic acid, and  
 about from 7% to 25% of an alkali metal base selected from the group consisting of sodium hydroxide and sodium carbonate, to a wet pickup of about 85-100%,  
 (b) curing the impregnated textile for about from 5 to 30 minutes at temperatures of about from 110° to 175° C., using the longer periods of time with the lower temperatures, then washing and drying the cured textile to obtain a finished produce with a phosphorus content of about from 0.06% to 1.58%.

11. A cellulosic derivative prepared according to the process of claim 10.

## 12

## References Cited

## UNITED STATES PATENTS

|           |         |                |           |
|-----------|---------|----------------|-----------|
| 2,971,815 | 2/1961  | Bullock et al. | 8-116 X   |
| 2,979,374 | 4/1961  | Drake et al.   | 8-116 X   |
| 3,110,727 | 11/1963 | Toy et al.     | 260-502.4 |

## OTHER REFERENCES

Marie, "Action de l'acide hypophosphoreux sur l'acetone," Comptes Rendus, 1901, pp. 219 to 221.

Moedritzer, "Synthesis and properties of phosphinic and phosphonic acid anhydrides," Journal of the American Chem. Soc., 1961, vol. 83, pp. 4381 to 4384.

WILLIAM D. MARTIN, Primary Examiner

HARRY J. GWINNELL, Assistant Examiner

## U.S. CL. X.R.

117—136, 137, 143